

## UNITED STATES PATENT OFFICE

2,482,142

## STRUCTURAL MATERIAL OF COMPRESSED RESIN IMPREGNATED PAPER SHEETS

Gardner H. Chidester, Parker K. Baird, George E. Mackin, Forrest A. Simmonds, Clarence O. Seborg, Mark W. Bray, and John N. McGovern, Madison, Wis.; dedicated to the free use of the People in the territory of the United States

No Drawing. Application October 2, 1943,  
Serial No. 504,780

6 Claims. (Cl. 154—45.9)

(Granted under the act of March 3, 1883, as amended April 30, 1928; 370 O. G. 757)

1

This application is made under the act of March 3, 1883, as amended by the act of April 30, 1928, and the invention herein described and claimed, if patented, may be manufactured and used by or for the Government of the United States of America for governmental purposes without the payment to us of any royalty thereon.

We hereby dedicate the invention herein described to the free use of the People in the territory of the United States to take effect on the granting of a patent to us.

This invention relates to structural materials and more particularly to such materials employing paper as a base, and a method of manufacturing them to impart high mechanical properties.

Laminated paper plastics have been made heretofore, but it has not been possible to manufacture them with sufficient strength to permit their use as structural parts of airplanes, automobiles, buildings, and so forth, that are subjected to high structural stresses. Paper laminated plastics of the prior art are limited in use generally to the taking of very light stresses and for decorative purposes.

We have found that by following a very careful procedure, paper laminated plastics can be made having enormous strength, being comparable on a weight basis to that of iron, aluminum, steel, and other structural materials, and in many respects more desirable.

In general, the process of our invention embraces cooking wood chips from species, such as black spruce, balsam fir or other suitable species yielding pulps making strong papers, to separate the fibers under such mild conditions that the original or native strength of the fibers is substantially preserved and not appreciably diminished. The sulfite, sulfate, or neutral sulfite process as ordinarily used to make chemical pulp in the pulp-making industry may be employed. When using the sulfite process, a relatively low temperature in the range of 120° C. to 135° C. and a relatively long period of time, namely, 10 to 20 hours, are used.

When the sulfate process is used, the total concentration of chemicals is relatively low (about 30 grams per liter) and the time of digestion is extended sufficiently to reduce completely the chips to pulp. However, lower or higher digestion temperatures and shorter cooking schedules may be used by adjusting the concentration of chemicals in the cooking liquor to about 50 to 70 grams per liter.

After cooking, the pulp, if beaten, is not proc-

essed more than to produce a degree of hydration sufficient to permit bonding of the fibers so that the fibers retain as much of their original or native strength as possible. Ordinarily, a hydration index of 750 to 850 cc. Schopper-Riegler freeness is sufficient. It is important to carefully observe this step in the process because the maximum strength cannot otherwise be developed in the plastic product. The fibers thus hydrated are then felted and dried to produce a sheet having high porosity, high density, and high tensile strength.

In producing the sheet, the specially prepared hydrated fibers are fed to the flow box of a paper machine at about 0.2 percent consistence and are flowed onto the Fourdrinier wire at a speed different from that of the wire, which results in alignment of the fibers in the direction of the flow thus producing a highly grained sheet. The difference in speed should be such as to obtain an anisotropy of grain which will provide a ratio of at least 2.0 to 1 in tensile strength. High sheet densities between 0.6 to 0.8 are obtained without materially reducing the porosity of the sheet by using very high pressures on the wet press (from 125 to 175 pounds per lineal inch of nip). Still further densification of the web may be accomplished by adjusting pressure on the calendars. The latter increases the strength but decreases the porosity of the sheet to a marked degree and, therefore, the use of high calendering pressure is limited to sheets of high porosity in the uncalendered condition.

The sheet should be formed very thin, generally less than 4 mils, in order to avoid the orientation of fibers in the third dimension (thickness). Ordinarily, a sheet of paper with a high degree of porosity has a correspondingly low tensile strength, and vice versa. The usual paper-making procedure for developing high porosity in paper is diametrically opposed to that for developing high tensile strength, generally achieved by hydrating the fibers, so that ordinarily a paper possessing one of these qualities to a high degree will possess the other quality to a very low degree. By following the process of this invention, a paper sheet is produced which has both high tensile strength and relatively high porosity. With such a paper, it is possible to fabricate laminated plastics with high structural strength under very low laminating pressures. In other words, the paper itself must be very strong and still be highly porous to permit thorough impregnation of the resin. In making the plastic, the paper is first impregnated with an uncured ther-

mosetting or thermoplastic resin, or a mixture of both, and then dried. The dried impregnated paper sheets are then assembled, with either the grain of the paper oriented parallel or alternately crosswise, and the resulting lamination cured under heat and low pressure to form the laminated paper plastic.

The following examples will illustrate this invention, but it is to be understood that they are not intended to limit in any way the scope thereof.

*Example 1*

Black spruce wood chips were cooked by the sulfate pulping process using a liquor of 33.85 percent sulfidity at a total concentration of 30 grams per liter and a total amount of chemicals equivalent to 20 percent of the moisture-free weight of the chips. The temperature of the mixture was raised from 35° C. to 170° C. during a period of 1½ hours and heating was continued at 170° C. for 3 hours. The pulp was then screened and beaten to a Schopper-Riegler freeness index of 835 cc. The beaten pulp was formed into a paper having a density of 0.61 gram per cc., a porosity index of 3.2 seconds, and a thickness of 2.6 mils. The paper had a tensile strength of 12,850 pounds per square inch in the machine direction and 4,670 pounds per square inch across the machine direction. The paper was then impregnated with an uncured phenol-formaldehyde resin and dried. Sheets of the impregnated paper were assembled in laminations, some with the grain laid in the parallel direction and others in crosswise directions. The laminations were then cured under a pressure of 250 pounds per square inch at a temperature 325° F. The resulting laminated plastics had the following properties when tested in grain for parallel laminates:

|                                             |                      |                     |
|---------------------------------------------|----------------------|---------------------|
| Tensile strength.....                       | 144,700 p. s. i.     | Parallel laminated. |
| Modulus of elasticity (in tension).....     | 128,020 p. s. i.     | Cross laminated.    |
| Modulus of rupture (in bending).....        | 133,396,000 p. s. i. | Parallel laminated. |
| Modulus of elasticity (in bending).....     | 12,046,000 p. s. i.  | Cross laminated.    |
| Compressive strength.....                   | 133,780 p. s. i.     | Parallel laminated. |
| Modulus of elasticity (in compression)..... | 130,415 p. s. i.     | Cross laminated.    |
| Modulus of elasticity (in compression)..... | 12,997,000 p. s. i.  | Parallel laminated. |
| Density.....                                | 11,953,000 p. s. i.  | Cross laminated.    |
|                                             | 25,280 p. s. i.      | Parallel laminated. |
|                                             | 2,920,000 p. s. i.   | Do.                 |
| Density.....                                | 11.39 grams per cc.  | Do.                 |
|                                             | 1.40 grams per cc.   | Cross laminated.    |

*Example 2*

Balsam fir wood chips were cooked by the sulfate pulping process using a liquor having 33.85 percent sulfidity, the total concentration of chemicals being 50 grams per liter. The temperature of the cooking was raised from 35° C. to 170° C. during a period of 1½ hours. The heating was continued at this temperature for 1½ hours. The pulp was then screened and beaten to a Schopper-Riegler freeness index of 845 cc. The beaten pulp was formed into a paper having a density of 0.62 gram per cc., a porosity index of 5.2 seconds, and a thickness of 2.6 mils. The paper had a tensile strength of 13,460 pounds per square inch in the machine direction and 4,680 pounds per square inch across the machine direction. The paper was then impregnated with an uncured phenol-formaldehyde resin and dried. Sheets of impregnated paper were assembled in laminations with the grain oriented in a parallel direction, and cured under a pressure of 250 pounds per square inch at a temperature of 350°

F. The resulting laminated plastic was found to have the following in grain properties:

|                                         |                                    |
|-----------------------------------------|------------------------------------|
| Tensile strength.....                   | 39,700 pounds per square inch..... |
| Modulus of elasticity (in tension)..... | 3,006,000 do.....                  |
| Modulus of rupture (in bending).....    | 36,960 do.....                     |
| Modulus of elasticity (in bending)..... | 2,731,000 do.....                  |
| Density.....                            | 1.35 grams per cc.....             |

*Example 3*

Same as Example 1, except that the initial concentration of the cooking liquor was increased from 30 to 70 grams per liter and the time of cooking at maximum temperature was decreased from 3 hours to 1 hour. The properties of the final parallel laminated plastic were as follows, when tested in grain:

|                                         |                                    |
|-----------------------------------------|------------------------------------|
| Tensile strength.....                   | 41,530 pounds per square inch..... |
| Modulus of elasticity (in tension)..... | 3,112,000 do.....                  |
| Modulus of rupture (in bending).....    | 33,060 do.....                     |
| Modulus of elasticity (in bending)..... | 2,984,000 do.....                  |
| Density.....                            | 1.32 grams per cc.....             |

*Example 4*

Same as Example 2, except that black spruce chips were used and the cooking was conducted over a period of 3 hours at a temperature of 160° C. The properties of the parallel laminated plastic were as follows, when tested in grain:

|                       |                                    |
|-----------------------|------------------------------------|
| Tensile strength..... | 38,790 pounds per square inch..... |
|-----------------------|------------------------------------|

*Example 5*

|                                         |                        |
|-----------------------------------------|------------------------|
| Modulus of elasticity (in tension)..... | 3,135,000 do.....      |
| Modulus of rupture (in bending).....    | 30,220 do.....         |
| Modulus of elasticity (in bending)..... | 2,672,000 do.....      |
| Density.....                            | 1.33 grams per cc..... |

Black spruce chips were cooked by the sulfite pulping process using 57.5 gallons of cooking liquor per 100 pounds of moisture-free wood, the liquor having a concentration of 6.0 percent total sulfur dioxide and 1.2 percent combined sulfur dioxide. The temperature of the mixture, after steaming the chips at atmospheric pressure for ½ hour prior to addition of the cooking liquor, was raised from 55° C. to 110° C. in 2 hours and held at 110° C. for 2 additional hours. The temperature was then increased to 130° C. during a period of 2 hours and finally, the heating continued at 130° C. for 4 hours. The resulting pulp after screening had a Schopper-Riegler freeness

index of 860 cc. The pulp without further treatment was formed into a paper having a density of 0.71 gram per cc., a porosity index of 12 seconds, and a thickness of 2.3 mils. The tensile strength of the paper was 13,860 pounds per square inch in the machine direction and 4,760 pounds per square inch across the machine direction. The paper was then impregnated with an uncured phenol-formaldehyde resin and dried. Sheets of impregnated paper were assembled in laminations with the grain of paper laid in a parallel direction, and cured under a pressure of 250 pounds per square inch at a temperature of 325° F. The resulting laminated plastic was found to have the following properties, when tested in grain for 15 parallel laminates:

|                       |          |                        |           |
|-----------------------|----------|------------------------|-----------|
| Tensile               | strength | pounds per square inch | 38,060    |
| Modulus of elasticity |          |                        | 3,474,000 |
| (in tension)          | do       | do                     | 3,474,000 |
| Modulus of rupture    |          |                        | 36,100    |
| (in bending)          | do       | do                     | 36,100    |
| Modulus of elasticity |          |                        | 3,293,000 |
| (in bending)          | do       | do                     | 3,293,000 |
| Density               |          | grams per cc           | 1.41      |

#### Example 6

Same as Example 5, except that a concentration of 5.25 percent total sulfur dioxide and 1.10 percent combined sulfur dioxide was used and the temperature was raised, after presteaming the chips, from 55° C. to 110° C. over a period of 2 hours and held at 110° C. for 2 hours; then raised to 120° C. in 1 hour; and finally heated at 120° C. for 10.25 hours. The Schopper-Riegler freeness index of the pulp after screening was 855 cc.

inch across the machine direction. The physical properties of the final resin-treated, parallel laminated plastic were as follows, when tested in grain:

|                       |         |              |                        |        |
|-----------------------|---------|--------------|------------------------|--------|
| 5                     | Tensile | strength     | pounds per square inch | 38,050 |
| Modulus of elasticity |         |              | 3,627,000              |        |
| (in tension)          | do      | do           | 3,627,000              |        |
| Modulus of rupture    |         |              | 31,930                 |        |
| (in bending)          | do      | do           | 31,930                 |        |
| Modulus of elasticity |         |              | 3,210,000              |        |
| (in bending)          | do      | do           | 3,210,000              |        |
| Density               |         | grams per cc | 1.41                   |        |

#### Example 8

Black spruce chips were cooked by the sulfite process using the same amount of liquor and concentration as in Example 6. The chips were presteamed and the temperature of the cooking mixture raised as described in Example 5. The resulting pulp was screened and beaten to a Schopper-Riegler freeness index of 858 cc. The beaten pulp was formed into paper having a density of 0.72 gram per cc., a porosity index of 13 seconds, and a thickness of 2.3 mils. The tensile strength of the paper was 14,480 pounds per square inch in the machine direction and 5,270 pounds per square inch across the machine direction. The paper was impregnated with uncured phenol-formaldehyde resin and dried. Sheets of impregnated paper were assembled in laminations, some with grain laid in parallel and others with grain laid in crosswise directions, and cured as in Example 5. The resulting laminated plastics had the following properties when tested in grain for 35 parallel laminates:

|                                    |  |                     |                     |
|------------------------------------|--|---------------------|---------------------|
| Tensile strength                   |  | 137,240 p. s. i.    | Parallel laminated. |
| Modulus of elasticity (in tension) |  | 125,480 p. s. i.    | Cross laminated.    |
| Modulus of elasticity (in bending) |  | 13,560,000 p. s. i. | Parallel laminated. |
| Modulus of rupture (in bending)    |  | 12,338,000 p. s. i. | Cross laminated.    |
| Modulus of elasticity (in bending) |  | 135,000 p. s. i.    | Parallel laminated. |
| Density                            |  | 126,935 p. s. i.    | Cross laminated.    |
|                                    |  | 13,400,000 p. s. i. | Parallel laminated. |
|                                    |  | 12,077,000 p. s. i. | Cross laminated.    |
|                                    |  | 1.41 grams per cc.  | Parallel laminated. |
|                                    |  | 1.39 grams per cc.  | Cross laminated.    |

#### Example 9

Balsam fir wood chips were cooked by the sulfite process for making chemical pulp using an amount of liquor equal to 62.5 gallons per 100 pounds of moisture-free wood, the liquor having the same concentration as in Example 5. The chips were steamed and the cooking temperature ranged the same as in Example 5, except that the heating was continued at 130° C. for 4.5 hours. The pulp was blown, screened and beaten to a Schopper-Riegler freeness index of 840 cc. and formed into paper having a density of 0.74 gram per cc., a porosity index of 75 seconds, and a thickness of 2.3 mils. The tensile strength of the paper in the machine direction was 14,350 pounds per square inch and 5,610 pounds per square inch across the machine direction. These sheets were then impregnated with uncured phenol-formaldehyde resin, dried, assembled, and cured the same as in Example 5. The resulting parallel laminated plastic had the following properties, when tested in grain:

|                       |         |          |                        |        |
|-----------------------|---------|----------|------------------------|--------|
| 70                    | Tensile | strength | pounds per square inch | 36,180 |
| Modulus of elasticity |         |          | 3,114,000              |        |
| (in tension)          | do      | do       | 3,114,000              |        |
| Modulus of rupture    |         |          | 35,330                 |        |
| (in bending)          | do      | do       | 35,330                 |        |

#### Example 7

Same as Example 6, except that the pulp was beaten to a Schopper-Riegler freeness index of 850 cc. The paper, made under the special paper making conditions, had a density of 0.74 gram per cc., a porosity index of 22 seconds, and a thickness of 2.3 mils. The tensile strength of the paper was 13,750 pounds per square inch in the machine direction and 4,950 pounds per square

Modulus of elasticity  
(in bending) ..... do ..... 3,010,000  
Density ..... grams per cc. .... 1.42

## Example 10

Black spruce wood chips were cooked by the neutral sulfite process for making chemical pulp, using an amount of liquor equal to 51.5 gallons per 100 pounds of moisture-free wood, the liquor having a concentration of 161 grams per liter of sodium sulfite. The liquor also contained a quantity of sodium sulfite equivalent to 2.5 percent of the wood on a moisture-free basis. The temperature of the cooking mixture was raised from 30° C. to 110° C. in 1 hour and then raised to 181° C. in 4.25 hours at which temperature the heating was continued for 3.75 hours. The pulp was formed into paper having a density of 0.67 gram per cc., a porosity index of 5 seconds, and a thickness of 2.0 mils. The tensile strength of the paper in the machine direction was 14,700 pounds per square inch and 5,570 pounds per square inch across the machine direction. The paper was then impregnated with an uncured phenol-formaldehyde resin and dried. Sheets of impregnated paper were assembled in both parallel and in crosswise laid laminations and cured at a pressure of 250 pounds per square inch at a temperature of 325° F. The resulting plastics had the following properties when tested in grain for parallel laminates:

|                                         |                                                  |                                                                |
|-----------------------------------------|--------------------------------------------------|----------------------------------------------------------------|
| Tensile strength.....                   | 44,590 p. s. i.....<br>27,900 p. s. i.....       | Parallel laminated.<br>Cross laminated.                        |
| Modulus of elasticity (in tension)..... | 3,225,000 p. s. i.....<br>3,225,000 p. s. i..... | Parallel laminated.<br>Cross laminated.                        |
| Modulus of rupture (in bending).....    | 32,600 p. s. i.....                              | Parallel laminated.                                            |
| Modulus of elasticity (in bending)..... | 2,975,000 p. s. i.....<br>(1.37 grams per cc.)   | Parallel laminated.<br>Parallel laminated.<br>Cross laminated. |
| Density.....                            | (1.38 grams per cc.)                             |                                                                |

Resins suitable for the production of high-strength laminates of paper include: Phenol-aldehyde resins (monohydric, dihydric, trihydric, and polyhydric phenols in combination with formaldehyde, benzaldehyde, furfuraldehyde, and other aldehydes, such as are obtained from aliphatic and aromatic acid compounds); amino-aldehydic resins, such as urea-aldehyde compounds, including thiourea and melamine-aldehyde resins; and other thermosetting resins having similar properties.

Paper laminated plastics of great mechanical strength result from the general fabrication process illustrated by the foregoing examples. Heretofore, it was not possible to obtain parallel-laminated paper plastics having tensile strengths of much over 20,000 pounds per square inch and correspondingly small moduli of elasticity, nor was it possible heretofore to obtain cross-laminated paper plastics having tensile strengths of more than 15,000 pounds per square inch, in grain, and correspondingly small moduli of elasticity. It is to be understood that any paper laminated plastic in which the grain direction of the laminations is parallel, generally referred to as parallel-laminated paper plastics having a tensile strength of over about 35,000 pounds per square inch and a modulus of elasticity in tension of over about 3,000,000 pounds per square inch, is within the scope of this invention. In the case of cross-laminated paper plastic materials, that is, where the grain direction of the paper laminations is alternated, those having a tensile strength of over about 25,000 pounds per square inch and a

modulus of elasticity of over about 2,000,000 pounds per square inch are within the scope of this invention.

Having thus described our invention, we claim:

1. A structural material comprising compressed synthetic resin-bonded laminated sheets of paper; each sheet being made from pulp having a freeness of 750 to 860 cc.; each sheet of paper having a porosity index of about 3.2 to 75 seconds, an anisotropy of grain providing a ratio of at least 2.0 to 1 in tensile strength, and a density of 0.60 to 0.80 gram per cc., and a thickness of not more than about 4 mils; said sheets having a distribution of a solid, strengthening synthetic resin in their porous structure which bonds them together; said structural material having a tensile strength of at least 25,000 lbs. per square inch and a modulus of elasticity in tension of over 2,000,000 pounds per square inch and having a density of not less than about 1.33.
2. The structural material defined in claim 1 in which the synthetic resin is a thermosetting resin.
3. The structural material defined in claim 1 in which the synthetic resin is a thermosetting phenol-formaldehyde resin.
4. The structural material defined in claim 1 in which the synthetic resin is a thermosetting phenol-aldehyde resin.
5. The structural material defined in claim 1

in which the synthetic resin is a thermosetting urea-aldehyde resin.

6. The structural material defined in claim 1 in which the synthetic resin is a thermosetting melamine-aldehyde resin.

GARDNER H. CHIDESTER.  
PARKER K. BAIRD.  
GEORGE E. MACKIN.  
FORREST A. SIMMONDS.  
CLARENCE O. SEBORG.  
MARK W. BRAY.  
JOHN N. McGOVERN.

## REFERENCES CITED

The following references are of record in the file of this patent:

## UNITED STATES PATENTS

| Number    | Name    | Date          |
|-----------|---------|---------------|
| 1,284,432 | O'Conor | Nov. 12, 1918 |
| 1,303,753 | Wright  | May 13, 1919  |

## FOREIGN PATENTS

| Number  | Country       | Date          |
|---------|---------------|---------------|
| 284,232 | Great Britain | Jan. 10, 1929 |

## OTHER REFERENCES

Modern Plastics Catalog, 1941, Design Div., pp. 394, 395.

Chemistry of Pulp and Papermaking (copy in Div. 56), Sutermeister, 3d ed., Chap. VI.

J. Wiley & Sons, N. Y., 1941, The Dictionary of Paper, Am. Paper and Pulp Assoc., 1940, p. 11. (Copy in Div. 56.)